

# United States Patent Office

2,861,907

Patented Nov. 25, 1958

1

2,861,907

## INHIBITION OF CORROSION OF METAL SURFACES BY SALT OF PHOSPHORODITHIOIC ACID

Thomas A. Butler, Cleveland, Ohio, assignor to The Lubrizol Corporation, Wickliffe, Ohio, a corporation of Ohio

No Drawing. Application September 28, 1956  
Serial No. 612,597

10 Claims. (Cl. 148—6.17)

This invention relates to a process for the inhibition of corrosion of metal surfaces and in particular to a process which is particularly useful for the inhibition of corrosion of ferrous metal surfaces.

The corrosion of metal surfaces is of obvious economic significance in many industrial applications, and as a consequence the inhibition of such corrosion is a matter of prime consideration in such applications. It is of particular significance to users of steel and other ferrous alloys. The corrosion of such ferrous metal alloys is largely a matter of rust formation which in turn involves the over-all conversion of the free metal to its oxide.

The theory which best explains such oxidation of ferrous metal surfaces postulates the essential presence both of water and oxygen. Even minute traces of moisture are sufficient, according to this theory, to induce the dissolution of iron therein until the water becomes saturated with iron ions. The presence of oxygen causes oxidation of the resulting ferrous hydroxide to ferric hydroxide which then settles out of solution and is ultimately converted to ferric oxide or rust.

The above sequence of reactions can be prevented, or at least in large measure inhibited, by relatively impermeable coatings which have the effect of excluding either or both moisture and oxygen from contact with the ferrous metal surfaces. Such coatings are, of course, subject to abrasion and other causes of physical deformation and to the extent that these coatings are penetrated or otherwise destroyed by such influences they are ineffective for the purpose desired. It is important that such coatings provide complete protection of all of the ferrous metal surfaces. If there is any portion of such a surface which is not so protected, regardless of how small the unprotected surface may be, the degree of protection afforded is considerably less than desirable. A satisfactory corrosion-inhibiting coating, then, must have the ability to resist substantial deformation upon impact, abrasion, etc. so that a uniform and complete film of protection is maintained in the face of such adverse influences.

It is accordingly a principal object of this invention to provide protection from corrosion for metal surfaces.

It is another object of this invention to provide protection from the formation of rust on ferrous metal surfaces.

Other objects will be apparent from the ensuing description.

These objects are achieved by the process of inhibiting corrosion of metal surfaces which comprises applying to said surfaces a film of a polyvalent metal salt of a phosphorodithioic acid prepared by the process which comprises

(a) The reaction of a mixture of a monohydric alcohol and from 0.25 to 4.0 equivalents of a polyhydric alcohol, with a phosphorus sulfide to form a phosphorodithioic acid, and

2

(b) Conversion of said acid to a polyvalent metal salt thereof.

It will be noted that the phosphorodithioic acid described above is a particular type of phosphorodithioic acid which is not readily characterized in terms of a structural formula. The structural formula which is characteristic of all phosphorodithioic acids is:



This formula, however, is not an entirely accurate representation of the phosphorodithioic acids of this invention because a substantial proportion of  $R_1$  and/or  $R_2$  is derived from a polyhydric alcohol. Consequently,  $R_1$ , for example, may be attached not only to the oxygen of the above structural formula but also to the oxygen of a second phosphorodithioic acid nucleus, or in the case of a trihydric alcohol reactant, to the oxygen of a third phosphorodithioic acid nucleus. Or it may be that  $R_1$  and  $R_2$  are the same alkylene radical, such alkylene radical being derived from a dihydric alcohol.

In view of the above-described difficulties in characterizing the phosphorodithioic acids of this invention in terms of a chemical structure, it is deemed best to describe these acids in terms of the process by which they may be prepared and, accordingly, they are described herein without reference to molecular structural formulas.

The monohydric alcohols contemplated as reactants in the process of this invention include principally the alkanols, although alcohols such as phenethyl and benzyl alcohols likewise may be used. For the most part, however, such alkanols as ethyl, butyl, hexyl, octyl, decyl, etc. alcohols are contemplated as the monohydric alcohol reactant. A particularly preferred subclass of monohydric alcohols are the octyl alcohols.

The polyhydric alcohol reactant may be selected from dihydric, trihydric and tetrahydric alcohols. Illustrative examples of such polyhydric alcohols include ethylene glycol, propylene glycol, butylene glycol, glycerol, pentaerythritol, butenediol, butynediol, etc. It is contemplated, likewise, to employ such polyhydric alcohols which may also contain aromatic substituents.

The proportions of monohydric and polyhydric alcohols which are to be used in the process of this invention are governed by considerations of solubility and fluidity on the one hand, and of satisfactorily permanent film-forming properties on the other hand. It has been found that the use of a disproportionately large amount of polyhydric alcohol in the reaction mixture results in a product which is too insoluble and intractable to allow of convenient application to a metal surface. If the proportion of polyhydric alcohol used in the reaction mixture is below a certain minimum quantity then the resulting product, although sufficiently fluid and soluble in many solvents, is not a satisfactory film-forming material, and coatings thereof applied to metallic surfaces do not afford a desirable degree of protection from corrosive influences. In view of these observations, it has been determined that the amount of polyhydric alcohol which can be used satisfactorily in the process here is within the range of 0.25 to 4.0 equivalents per equivalent of monohydric alcohol present in the reaction mass. It is particularly preferred to employ approximately equivalent amounts of monohydric and polyhydric alcohol reactants.

The term "equivalent," as used above is based upon a consideration of the number of hydroxyl groups in the particular alcohol reactant. Thus the equivalent weight of ethylene glycol is 31, one-half of the molecular weight

thereof. The equivalent weight of pentaerythritol is 34, one-fourth the molecular weight thereof. In view of the principal reaction of the process, i. e., phosphorus pentasulfide with the alcohols, it is evident that the relative quantities of alcohol reactants must in this case be discussed in terms of their equivalent weights.

The reaction by which phosphorodithioic acids are prepared is well known. It involves the reaction of one mole of phosphorus pentasulfide with four equivalents of an alcohol. In any discussion of the process of this invention, it is understood that this ratio of reactants is to be employed.

Although other phosphorus sulfides may be used, it is preferred both for reasons of economy and efficacy of reaction to use phosphorus pentasulfide.

The metal constituent of the corrosion-inhibiting agent of this invention is polyvalent. The divalent metals are preferred, and of these zinc is particularly desirable. These metal salts are prepared from the phosphorodithioic acid, generally by neutralization thereof with the particular basic metal compound of the desired metal. Thus the preparation of a zinc phosphorodithioate may be effected by neutralization of the phosphorodithioic acid with zinc oxide. Similarly, a barium salt may be prepared by neutralization with barium hydroxide octahydrate. Other methods of formation of such polyvalent metal salts may be accomplished by reaction of the phosphorodithioic acid with the free metal, such as metallic calcium.

The process by which these polyvalent metal salts are prepared is illustrated in detail by the following examples:

*Example 1.*—To a solution of 1040 grams (8 equivalents) of n-octyl alcohol in 304 grams (8 equivalents) of 1,2-propylene glycol there was added over a period of 2 hours at 60-70° C., 888 grams (4 moles) of phosphorus pentasulfide. The mixture was heated at 70-75° C. for 3 hours and filtered. A portion of the filtrate, weighing 678 grams (2 moles), was added slowly with stirring to a mixture of 89 grams (1.1 moles) of zinc oxide and 741 grams of toluene. This mixture was filtered to yield a filtrate having the following analyses:

Percent P..... 5.0  
Percent S..... 9.9  
Percent Zn..... 4.8

*Example 2.*—A solution of 520 grams (4 equivalents) of isooctyl alcohol, 180 grams (4 equivalents) of 2-butent-1,4-diol in 1106 grams of toluene was prepared and treated with 444 grams (2 moles) of phosphorus pentasulfide. The resulting mixture was heated at 42-60° C. for 7 hours, then filtered. To 2000 grams (3.28 moles) of the filtrate there was added at 60-65° C., 147 grams (180 moles) of zinc oxide. The mixture was heated up to 115° C. over a 2-hour period by which time 31 grams of water had been removed by distillation. The residue was filtered to yield a filtrate having the following analyses:

Percent P..... 5.3  
Percent S..... 10.7  
Percent Zn..... 5.4

*Example 3.*—To a solution of 382 grams (2.94 equivalents) of isooctyl alcohol and 131 grams (2.94 equivalents) of 2-butyne-1,4-diol in 789 grams of toluene there was added 326 grams (1.45 moles) of phosphorus pentasulfide. This mixture was heated at 75-85° C. for 2 hours, then filtered. To 1150 grams (1.23 moles) of the filtrate there was added at 60-65° C. 55 grams (0.68 mole) of zinc oxide. The mixture was heated at 115° C. for 2 hours, removing 9 grams of water. The residue was filtered to yield a filtrate having the following analyses:

Percent P..... 3.6  
Percent S..... 8.1  
Percent Zn..... 3.6

*Example 4.*—To a mixture of 650 grams (5.0 equivalents) of isooctyl alcohol and 1010 grams (15.0 equivalents) of dipropylene glycol there was added 1110 grams (5.0 moles) of phosphorus pentasulfide. The resulting mass was heated at 70-80° C. for 2 hours and filtered. To a solution of 290 grams (1.0 mole) of the filtrate in 740 grams of isopropanol there was added 45.5 grams (0.55 mole) of zinc oxide. This mixture was heated at 45° C. for 3.5 hours, then filtered. The filtrate showed the following analyses:

Percent P..... 3.6  
Percent S..... 7.2  
Percent Zn..... 2.8

*Example 5.*—A mixture of 1560 grams (12 equivalents) of isooctyl alcohol, 808 grams (12 equivalents) of dipropylene glycol and 1332 grams (6 moles) of phosphorus pentasulfide was heated at 65-70° C. for 4 hours and filtered. To 500 grams (1.58 moles) of the filtrate there was added 70.9 grams (0.87 mole) of zinc oxide, and 550 grams of n-butyl alcohol. The mixture was stirred briefly and then filtered to yield a clear solution having the following analyses:

Percent P..... 4.5  
Percent S..... 9.3  
Percent Zn..... 4.5

*Example 6.*—A mixture of 740 grams (10 equivalents) of n-butyl alcohol, 531 grams (10 equivalents) of diethylene glycol and 1110 grams (5 moles) of phosphorus pentasulfide was heated at 70-75° C. for 3 hours, and then filtered. A portion of the filtrate weighing 504 grams (2 moles) was added slowly to a suspension of 89.6 grams (1.06 moles) of zinc oxide in 1000 grams of toluene. This mixture was heated at 40-80° C./25 mm. for 2 hours and filtered. The filtrate showed the following analyses:

Percent P..... 4.9  
Percent S..... 10.5  
Percent Zn..... 4.9

*Example 7.*—To a mixture of 1116 grams (6 equivalents) of a mixture of C<sub>12</sub> alcohols and 319 grams (6 equivalents) of diethylene glycol there was added portionwise at 60-70° C. 666 grams (3 moles) of phosphorus pentasulfide. The resulting mixture was heated for an additional 2 hours at 70-75° C. and then filtered. A portion of the filtrate weighing 776 grams (2 moles) was added slowly to a suspension of 89 grams (1.1 moles) of zinc oxide in toluene. The mixture was heated at 40-60° C./25 mm. for 4 hours during which time 18 grams of water was collected. The residue was filtered and the filtrate had the following analyses:

Percent P..... 3.9  
Percent S..... 7.6  
Percent Zn..... 3.9

*Example 8.*—A mixture of 1560 grams (12 equivalents) of isooctyl alcohol, 808 grams (12 equivalents) of dipropylene glycol and 1332 grams (6 moles) of phosphorus pentasulfide was heated at 50° C. for 3 hours and then filtered. To 584 grams (1 mole) of the filtrate dissolved in 640 grams of toluene there was added at 55° C. 66 grams (1.18 moles) of iron filings. The resulting mixture was heated at 60° C. for 10 hours and filtered. The filtrate was analyzed and found to have the following:

Percent P..... 4.9  
Percent S..... 9.6  
Percent Fe..... 1.5

*Example 9.*—A mixture of 975 grams (7.5 equivalents) of n-octyl alcohol, 186 grams (6 equivalents) of di-

ethylene glycol, 47 grams (1.5 equivalents) of glycerol and 833 grams (3.75 moles) of phosphorus pentasulfide was heated for 4 hours at 70-75° C. and then filtered. A portion of the filtrate weighing 722 grams (2 moles) was added portionwise to a suspension of 89 grams (1.1 moles) of zinc oxide in 785 grams of toluene. The resulting mixture was stirred vigorously and then dehydrated by heating at 40-60° C./20 mm. for 2.5 hours. The residue was filtered; the filtrate showed the following analyses:

|            |     |
|------------|-----|
| Percent P  | 4.8 |
| Percent S  | 9.5 |
| Percent Zn | 4.9 |

*Example 10.*—To a mixture of 1040 grams (8 equivalents) of isoctyl alcohol and 246 grams (8 equivalents) of glycerol there was added 88 grams (4 moles) of phosphorus pentasulfide. This mixture was heated at 70-75° C. for 4 hours and then filtered. To a suspension of 89 grams (1.1 moles) of zinc oxide in 775 grams of toluene there was added slowly 712 grams (2 moles) of the resulting phosphorodithioic acid (filtrate). This neutralization mixture was heated at 40-80° C./20 mm. for 2 hours and then filtered. The filtrate showed the following analyses:

|            |     |
|------------|-----|
| Percent P  | 4.5 |
| Percent S  | 8.5 |
| Percent Zn | 4.4 |

*Example 11.*—A mixture of 1040 grams (8 equivalents) of isoctyl alcohol and 68 grams (2 equivalents) of pentaerythritol and 555 grams (2.5 moles) of phosphorus pentasulfide was heated at 75-102° C. for 4 hours and then filtered. To a solution of 461 grams (3.94 moles) of the resulting phosphorodithioic acid in 1585 grams of toluene there was added portionwise 177 grams (2.18 moles) of zinc oxide. This mixture was heated at 75-80° C. for 2 hours and then filtered. The filtrate was analyzed and showed the following:

|            |     |
|------------|-----|
| Percent P  | 4.2 |
| Percent S  | 7.7 |
| Percent Zn | 4.2 |

*Example 12.*—A mixture of 1560 grams (12 equivalents) of isoctyl alcohol, 373 grams (12 equivalents) of diethylene glycol and 1332 grams (6 moles) of phosphorus pentasulfide was heated at 50-70° C. for 2 hours and then filtered. A portion of this phosphorodithioic acid filtrate weighing 1120 grams (4 moles) was heated at reflux temperature for 3 hours with 89 grams (4.94 equivalents) of water. A portion of the resulting product, a phosphoromonothioic acid, weighing 793 grams (3.0 moles) was added slowly and with stirring to a suspension of 128 grams (1.57 moles) of zinc oxide in 893 grams of toluene. This resulting mixture was heated at 50° C./20 mm. for 2 hours. Filtration of the residue yielded a toluene solution having the following analyses:

|            |     |
|------------|-----|
| Percent P  | 4.8 |
| Percent S  | 6.5 |
| Percent Zn | 5.7 |

*Example 13.*—A mixture of 520 grams (10 equivalents) of neopentyl glycol (2,2-dimethylpropane-1,3-diol), 1300 grams (10 equivalents) of isoctyl alcohol and 1110 grams (5 moles) of phosphorus pentasulfide was heated at 80-85° C. for 2 hours and filtered. A solution of 1734 grams (5.7 moles) of the filtrate in 1900 grams of toluene was treated portionwise at 75-80° C. and with stirring with 284 grams (3.97 moles) of zinc oxide. This mixture was heated for an additional 2 hours at 75° C. and again for another hour at 99-120°

C. The mixture was then filtered to yield a toluene solution having the following analyses:

|            |     |
|------------|-----|
| Percent P  | 4.6 |
| Percent S  | 9.1 |
| Percent Zn | 5.4 |

*Example 14.*—To a mixture of 520 grams (4 equivalents) of isoctyl alcohol and 632 grams (4 equivalents) of 2,2-bis(4-beta-hydroxyethoxyphenyl)propane there

10 was added 440 grams (2 moles) of phosphorus pentasulfide. This mixture was heated at 70-80° C. for 2 hours and filtered. A solution of 1156 grams (3 moles) of this filtrate in 600 grams of toluene was added to a suspension of 134 grams (1.65 moles) of zinc oxide in 2298 grams of toluene at 70-80° C. The mixture was heated at this temperature for an additional 3 hours and then filtered. The filtrate showed the following analyses:

|            |     |
|------------|-----|
| Percent P  | 2.0 |
| Percent S  | 3.9 |
| Percent Zn | 1.9 |

*Example 15.*—A phosphorodithioic acid was prepared in Example 12 and 584 grams thereof (2 moles) was added to a suspension of 190 grams (1.1 moles) of barium hydroxide in toluene. The resulting mixture was heated at 55-60° C. for 2 hours and then 55-60° C./20 mm. The residue showed the following analyses:

|            |     |
|------------|-----|
| Percent P  | 3.9 |
| Percent S  | 7.5 |
| Percent Ba | 9.0 |

*Example 16.*—A phosphorodithioic acid was prepared as in Example 8 and to 500 grams (1.58 moles) thereof dissolved in 500 grams of isopropyl alcohol at 50-60° C. there was added 31.6 grams (0.79 mole) of calcium metal turnings. The resulting mixture was heated at reflux temperature for 6 hours and then filtered. The resulting solution showed the following analyses:

|            |      |
|------------|------|
| Percent P  | 5.0  |
| Percent S  | 10.3 |
| Percent Ca | 2.8  |

*Example 17.*—A mixture of 1040 grams (8 equivalents) of isoctyl alcohol, 304 grams (8 equivalents) of propylene glycol and 888 grams (4 moles) of phosphorus pentasulfide was heated at 70-75° C. for 3 hours and filtered. A mixture of 300 grams (1 mole) of this filtrate, 67.5 grams (0.58 mole) of cadmium oxide, 100 grams of benzene and 355 grams of isopropyl alcohol was heated at 40° C. for 2 hours, and then filtered. The filtrate showed the following analyses:

|            |     |
|------------|-----|
| Percent P  | 4.5 |
| Percent S  | 9.2 |
| Percent Cd | 8.3 |

*Example 18.*—To a mixture of 118 grams (0.53 mole) of lead monoxide, 201 grams of benzene and 402 grams of isopropyl alcohol there was added 300 grams (1 mole) of the phosphorodithioic acid prepared as in Example 17. This mixture was heated at 35-45° C. for 3 hours and then filtered. The filtrate had the following analyses:

|            |      |
|------------|------|
| Percent P  | 3.9  |
| Percent S  | 7.5  |
| Percent Pb | 10.9 |

The corrosion inhibiting compositions exemplified by the products of the above examples are usually applied to a metallic surface as a solution in an inert solvent. Such solvents ideally are sufficiently volatile so as to allow their ready removal at convenient temperatures. Suitable solvents for this purpose include xylene, toluene, benzene, diethyl ether, alcohols, etc. In some instances the corrosion inhibitors may be applied as such, i. e., without a solvent, and in still others it is advantageous to apply them in aqueous emulsions. The method of application, like

7  
wise, is variable. Spraying, brushing and dipping are all acceptable methods.

The effectiveness of the film which is deposited on the metal surface depends upon the impermeability of the film to the corrosive influences which would otherwise be brought to bear upon the metal surface. This effectiveness, likewise, is dependent upon the prolonged resistance of the film to deformation or destruction upon impact, abrasion, etc. In view of the properties of the corrosion inhibiting composition of this invention, it is 5 apparent that these compositions are readily adaptable to provide protection against corrosion to all metal surfaces. Because of the peculiar susceptibility of iron to the moisture and oxygen content of the atmosphere, these compositions are especially valuable as protective films on ferrous metal surfaces.

The protection of ferrous metal surfaces from corrosion may be accomplished in part not only by protective films, but also by a phenomenon known as passivation. According to this latter method the ferrous metal surface is treated with a passivating agent such as nitric acid or phosphoric acid. A brief reaction ensues after which the metal is then less susceptible to corrosion; it is "passivated." A particularly useful method of passivating involves the treatment of a ferrous metal surface with a "phosphating" solution. Such phosphating solutions impart a degree of protection from corrosion by virtue of their ability to render a ferrous metal surface less susceptible to the formation of rust than it was previously.

It has been observed that an unusually high degree of protection from corrosion can be imparted to a ferrous metal surface by utilizing a combination of such a phosphating treatment together with the application of a film of the corrosion preventing composition of this invention. The net effect of such a combination has been demonstrated to be considerably in excess of the additive effects of each of these measures when used alone.

The effectiveness of the polyvalent metal phosphorothioates, described herein, as corrosion preventing agents for metal surfaces has been demonstrated by means of a "Salt Fog Test." This test (ASTM (1954), B-117-54T) involves the dipping of 3" x 3" steel panels into a solution of the sample to be tested. The panels are withdrawn at a specified rate so as to insure a uniformly thick film. The solvent is allowed to evaporate, and then the edges of the panels are painted with an air-drying enamel so as to assist in the reproducibility of the corrosion test to be carried out. Then the panels are placed in an enclosed cabinet which contains a 5 percent aqueous solution of sodium chloride at 95° C. This sodium chloride solution is agitated by means of a vigorous stream of air bubbled through the solution so as to produce a corrosive salt-steam atmosphere in the cabinet. The resistance of the panels to corrosion is measured in terms of the time required to produce a single rust spot on the panel in this atmosphere. It is apparent that the degree of protection from corrosion will be related to the thickness of the film which is deposited upon the metal surface, so that any numerical measure of protection from corrosion must take into account this factor of film thickness. Accordingly, the thickness of the film is expressed in terms of milligrams (of film) per square foot (of metal surface area). The use of this expression allows an evaluation of the effectiveness of the corrosion preventing films of this invention in terms of "hours (of 45 rust-free exposure in a salt-steam atmosphere), per milligrams (of film), per square foot (of metal surface area)." In order to facilitate the comparison of these values for different films the "salt-fog life" described above has been expressed as "hours/250 mg./ft.<sup>2</sup>".

The effectiveness of the metal salts of this invention as film-forming inhibitors of corrosion is shown by the table below in which each "salt-fog life" represents an average of results from six separate steel panels containing films of different thicknesses.

| Metal phosphorothioate                                                                                                                             | Salt-fog life (hours/250 mg./ft. <sup>2</sup> ) |
|----------------------------------------------------------------------------------------------------------------------------------------------------|-------------------------------------------------|
| 1. Zinc salt of phosphorodithioic acid prepared by reaction of $P_2S_4$ with $i-C_8H_{17}OH$ and pentaerythritol (4:1 equivalent ratio)            | 3.1                                             |
| 2. Zinc salt of phosphorodithioic acid prepared by reaction of $P_2S_4$ with lrol <sup>1</sup> and diethylene glycol (1:1 equivalent ratio)        | 2.5                                             |
| 3. Zinc salt of phosphorodithioic acid prepared by reaction of $P_2S_4$ with $n-C_8H_{17}OH$ and propylene glycol (1:1 equivalent ratio)           | 3.0                                             |
| 4. Zinc salt of phosphorodithioic acid prepared by reaction of $P_2S_4$ with $n-C_8H_{17}OH$ ethylene glycol and glycerol (5:4:1 equivalent ratio) | 3.9                                             |
| 5. Zinc salt of phosphoromothioic acid prepared from $i-C_8H_{17}OH$ and ethylene glycol (1:1 equivalent)                                          | 3.0                                             |
| 6. Uncoated steel panel                                                                                                                            |                                                 |

<sup>1</sup> Commercial mixture of  $C_{12}$  alcohols obtained by hydrogenation of coconut oil.

The data of the above table indicates the effectiveness of the film-forming compositions described herein. As indicated previously, however, the effectiveness of these compositions is even more striking when applied to metal surfaces which have previously been "passivated." This is shown by data obtained by the treatment of phosphated ferrous surfaces with various compositions of the type described herein. The method of phosphating the ferrous surfaces comprised immersing steel panels for 6 minutes in a solution containing 1.6 moles of phosphoric acid ( $H_3PO_4$ ), 0.4 mole of mono-ammonium phosphate ( $NH_4H_2PO_4$ ), 1 mole of zinc nitrate ( $Zn(NO_3)_2$ ), and 1 mole of calcium nitrate ( $Ca(NO_3)_2$ ) at 180-190° F. The panels are removed, rinsed with hot water, and then with dilute chromic acid (0.5 gram/liter) at 180-190° F. After drying the panels are ready to be coated with the corrosion-inhibiting compositions of this invention in the manner described previously. The results of salt-fog life determinations of steel panels which have been phosphated and then coated with the polyvalent metal phosphorothioates of this invention are shown in the following table.

Table II

| Rust-proofing composition | Salt-fog life (hours/250 mg./ft. <sup>2</sup> ) |
|---------------------------|-------------------------------------------------|
| None                      | 6                                               |
| Product of Example 1      | 1 681                                           |
| Product of Example 2      | 516                                             |
| Product of Example 3      | 499                                             |
| Product of Example 4      | 1 83                                            |
| Product of Example 5      | 464                                             |
| Product of Example 6      | 1 100                                           |
| Product of Example 7      | 1 257                                           |
| Product of Example 8      | 179                                             |
| Product of Example 9      | 1 390                                           |
| Product of Example 10     | 1 545                                           |
| Product of Example 11     | 421                                             |
| Product of Example 12     | 310                                             |
| Product of Example 13     | 1 250                                           |
| Product of Example 14     | 1 96                                            |
| Product of Example 15     | 1 69                                            |
| Product of Example 16     | 48                                              |
| Product of Example 17     | 1 59                                            |
| Product of Example 18     | 1 46                                            |

<sup>1</sup> Edges of the test specimens have been painted with an air-drying enamel.

65 Another principal application of the compositions of this invention depends upon its utility as a primer for metal surfaces, particularly those which have been phosphated or otherwise pre-treated. As a primer the metal salts of this invention not only afford a high degree of protection from corrosion but serve also to provide a relatively permanent bond between the metal surface and the outside enamel coating.

70 Other modes of applying the principle of the invention may be employed, change being made as regards the details described, provided the features stated in any of

the following claims or the equivalent of such be employed.

I, therefore, particularly point out and distinctly claim as my invention:

1. The process of inhibiting corrosion of metal surfaces which comprises applying to said surfaces a film of a polyvalent metal salt of a phosphorodithioic acid prepared by the process which comprises (a) the reaction of a mixture of a monohydric alcohol and from 0.25 to 4.0 equivalents of a polyhydric alcohol, with a phosphorus sulfide to form a phosphorodithioic acid, and (b) conversion of said acid to a polyvalent metal salt thereof.

2. The process of claim 1 characterized further in that said metal surfaces are treated, prior to the application of said polyvalent metal salt, with a phosphating solution.

3. The process of claim 1 characterized further in that the monohydric alcohol of (a) is an octyl alcohol.

4. The process of claim 1 characterized further in 20 that the monohydric alcohol of (a) is isoctyl alcohol.

5. The process of claim 1 characterized further in that the polyhydric alcohol of (a) is propylene glycol.

6. The process of claim 1 characterized further in 25 that the polyhydric alcohol of (a) is dipropylene glycol.

7. The process of claim 1 characterized further in that the polyvalent metal salt is a zinc salt.

8. The process of inhibiting corrosion of metal surfaces which comprises applying to said surfaces a film of a zinc salt of a phosphorodithioic acid prepared by the process which comprises (a) the reaction of a mixture of a monohydric alcohol and an approximately equivalent amount of polyhydric alcohol, with phosphorus pentasulfide to form a phosphorodithioic acid and (b) conversion of said phosphorodithioic acid to the zinc salt thereof by reaction with zinc oxide.

9. The process of claim 8 characterized further in that the metal surfaces are ferrous metal surfaces.

10. The process of claim 9 characterized further in 15 that said ferrous metal surfaces are treated, prior to the application of said zinc salt, with a phosphating solution.

References Cited in the file of this patent

UNITED STATES PATENTS

|           |                 |               |
|-----------|-----------------|---------------|
| 2,063,629 | Salzberg        | Dec. 8, 1936  |
| 2,564,864 | Thompson        | Aug. 21, 1951 |
| 2,671,758 | Vinograd et al. | Mar. 9, 1954  |